

B. F. RICHARDSON.  
COMPOSITION ROADWAY.  
APPLICATION FILED OCT. 13, 1908.

911,445.

Patented Feb. 2, 1909.



Witnesses:-

*Titus H. Jones.*  
*Augustus B. Oppen*

Iruevitor:-  
Benjamin F. Richardson  
by his Attorneys:  
*Howard & Sonnen*

# UNITED STATES PATENT OFFICE.

BENJAMIN F. RICHARDSON, OF PHILADELPHIA, PENNSYLVANIA, ASSIGNOR TO THE FELBERT PAVING AND CONSTRUCTION COMPANY, OF WILMINGTON, DELAWARE, A CORPORATION OF DELAWARE.

## COMPOSITION ROADWAY.

No. 911,445.

Specification of Letters Patent.

Patented Feb. 2, 1909.

Application filed October 13, 1908. Serial No. 457,492.

*To all whom it may concern:*

Be it known that I, BENJAMIN F. RICHARDSON, a citizen of the United States, residing in Philadelphia, Pennsylvania, have invented certain Improvements in Composition Roadways, of which the following is a specification.

My invention relates to certain improvements in the method of resurfacing old Macadam or Telford roadways.

One object of my invention is to provide a road surface which will be equal to the original surface of the road and which will be waterproof so as to prevent the accumulation 15 of water below the surface of the road and insure a more stable surface than has heretofore been obtained.

My invention also relates to certain improvements in the water proof composition 20 which I use in re-surfacing a road.

The figure in the accompanying drawing is a sectional view showing a portion of a road resurfaced according to my invention.

Referring to the drawing, A illustrates the 25 old road-bed, B a layer of asphalt cement, C a layer of crushed stone and D a layer of stone screenings.

In re-surfacing a Macadam or Telford road all dirt and refuse matter on the old roadway 30 is first removed and whenever the roadway is out of contour it must be brought to grade either by reducing the high points or by adding to the low points, while the ruts may be filled with crushed stone of  $1\frac{1}{2}$  inch gage 35 down to  $1/10$  of an inch gage, in order to bring the grade and crown of the road to the proper height, as the case may be.

After the above operations have been finished, the roadway is thoroughly compacted 40 by rolling, and for this purpose I prefer to use a steam roller of not less than five tons in weight, although such weight will depend materially upon the character of the roadbed.

I then coat this prepared surface while dry 45 with a waterproof asphalt cement to an approximate average depth of  $\frac{1}{4}$  of an inch. The asphalt cement is applied while hot and it may be either sprinkled or poured onto the surface though it may be applied by brooming or by other suitable means. This asphalt cement is composed of bitumen consisting of natural hydrocarbons and suitable fluxes for giving it a consistency suitable for paving purposes. The percentage of bitumen 50 soluble in carbon bi-sulfid shall in no

event fall below ninety and shall not be affected by the action of water. It must not oxidize nor be susceptible to atmospheric influences. Upon this layer of asphalt cement I apply crushed hard stone, preferably trap rock. Such stone must be of such size as to pass through a three-quarter inch mesh and must be dry when applied. This stone surface should be about one inch in thickness, thoroughly compacted by rolling, and the 65 roller should not be less than five tons in weight. Upon this layer will be placed one-half inch of evenly spread dry stone screenings (trap rock screenings being preferred) and this final wearing surface should also be 70 thoroughly compacted by the use of a roller. In no case should free asphalt cement appear upon the surface. After the bed has sufficiently cooled the road can be thrown open to the public.

By the above process of making a pavement I am enabled to re-surface an old Macadam or Telford road with a hard waterproof surface, which will withstand considerable wear and through which water will be unable 80 to pass, thus making a road-bed which will be very substantial.

I claim:

1. The process herein described of re-surfacing Macadam or Telford roads, said process consisting in first cleaning the surface of the old roadway and bringing it to the grade and crown desired by rolling, then applying to the prepared surface one-quarter inch thickness of hot asphalt cement, then applying broken stone of about one inch thickness, rolling said stone surface, then applying screenings to about one-half inch in thickness, and finally rolling the surface of screenings so as to produce a smooth roadway with 95 the proper crown and thoroughly compact the stones and screenings.

2. The process herein described of re-surfacing a roadway, said process consisting in preparing the old roadway so as to give it the 100 proper grade and crown, then applying an asphalt cement consisting of bitumen composed of natural hydrocarbons and suitable fluxes, the percentage of bitumen soluble in carbon bi-sulfid in no event falling below 105 ninety, placing upon the coating of asphalt cement a wearing surface composed of three-quarter inch dry crushed stone to a thickness of one inch, thoroughly compacting the said layer by rolling, evenly spreading thereon 110

one-half inch of dry stone screenings, and finally thoroughly compacting this surface by rolling, the stone being laid to prevent the appearance of free asphalt cement upon the surface.

3. The process herein described of re-surfacing Macadam or Telford roads, said process consisting in first cleaning the surface of the old roadway and bringing it to the grade and crown desired by rolling, then applying to the prepared surface a layer of asphalt cement, then applying a layer of broken stone rolling said stone surface, then apply-

ing a layer of screenings and finally rolling the surface of screenings so as to produce a smooth roadway with the proper crown and thoroughly compact the stones and screenings.

In testimony whereof, I have signed my name to this specification, in the presence of two subscribing witnesses.

BENJAMIN F. RICHARDSON.

Witnesses:

HENRY A. SHELDON,  
J. RALPH NAGLE.